

Feb. 27, 1951

G. N. JEPSSON

2,543,549

REFRACTORY SUPPORT FOR WARE IN A TUNNEL KILN

Filed Oct. 30, 1948

2 Sheets-Sheet 1



*Fig. 1*



*Fig. 2*



*Fig. 3*

INVENTOR

GEORGE N. JEPSSON

By *George Jeppson Jr.*  
ATTORNEY

Feb. 27, 1951

G. N. JEPSON

2,543,549

## REFRACTORY SUPPORT FOR WARE IN A TUNNEL KILN

Filed Oct. 30, 1948

2 Sheets-Sheet 2



Fig. 4



Fig. 5

INVENTOR

## GEORGE N. JEPSON

By George C. Crompton Jr.  
ATTORNEY

## UNITED STATES PATENT OFFICE

2,543,549

REFRACTORY SUPPORT FOR WARE IN A  
TUNNEL KILNGeorge N. Jeppson, Worcester, Mass., assignor to  
Norton Company, Worcester, Mass., a corpora-  
tion of Massachusetts

Application October 30, 1948, Serial No. 57,511

7 Claims. (Cl. 25—153)

1

The invention relates to refractory supports for ware in a tunnel kiln.

One object of the invention is to provide a refractory support for ware in a tunnel kiln which has a fast heating and cooling cycle. Another object of the invention is to provide a system of batts to support a grinding wheel being vitrified in a tunnel kiln of such construction and arrangement that the batts may be mechanically propelled through the kiln without the use of cars or movable elements other than the batts themselves and whereby a rapid vitrifying and annealing cycle may be achieved without excessive breakage of the batts due to thermal shock or otherwise. Another object of the invention is to provide a sliding batt construction especially adapted for the vitrification of large grinding wheels in a fast heating cycle. Another object of the invention is to provide a support for large articles to be vitrified in a tunnel kiln having planes of radiant energy above and below the support.

Other objects will be in part obvious or in part pointed out hereinafter.

The invention accordingly consists in the features of construction, combinations of elements and arrangements of parts, all as will be illustratively described herein and the scope of the application of which will be indicated in the following claims.

In the accompanying drawings illustrating one of many possible embodiments of the mechanical features of this invention,

Figure 1 is a plan view showing a plurality of batt elements supporting a single large grinding wheel to be vitrified and illustrating the rods upon which the batts slide.

Figure 2 is a cross sectional view taken on the line 2—2 of Figure 1.

Figure 3 is a cross sectional view taken on the line 3—3 of Figure 1.

Figure 4 is a longitudinal sectional view through a portion of the heating or firing zone of a tunnel kiln in which the refractory support of the invention may be used showing such refractory support in section.

Figure 5 is a cross sectional view of the kiln and support, the section being taken on the line 5—5 of Figure 4.

Referring first to Figures 1, 2 and 3, in this illustrative embodiment of the invention, a unit which is moved through the kiln comprises four batts 30 which straddle the tunnel and slide on rods 31, six batts 32 which rest upon the batts 30 and extend parallel to the rods 31, four end baffles 33, two center baffles 34 and a grinding wheel to be vitrified 35. Preferably a layer of quartz sand or the like 35a is placed on top of the longitudinally extending batts and the grinding wheel 35 rests upon this layer. The baffles 33 and

2

34 may rest upon the longitudinally extending batts 32. The purpose of the baffles 33 and 34 is to form with the roof and sidewalls of the tunnel and the batts 30 and 32 a compartment for each grinding wheel as it is being preheated, as it is being fired, and as it is being annealed. These baffles accordingly have curved edges as shown. A pair of baffles 33 with a center baffle 34 form a segmental wall following the contour of part of the periphery of the grinding wheel 35. By using three pieces to form each baffle means ahead of and behind the grinding wheel, fracturing of such baffle means due to heat shock or thermal differential is substantially eliminated.

Likewise the lower support for the grinding wheel 35 consists of four narrow batts 30 instead of a single batt in order that thermal differentials will be less liable to cause fracture. The upper support for the grinding wheel 35 consists of six batts 32 for the same reason. Each batt therefore is long in one dimension and relatively narrow. I have found that narrow batts will withstand a great many cycles of heating and cooling whereas more or less square batts have a greater tendency to break when subjected to repeated cycles of heating and cooling.

Also by forming the batt support for the wheels in two layers of batts, that is to say a lower layer of batts 30 and an upper layer of batts 32, I provide a support which will withstand many more cycles of heating and cooling than if the batt or batts were in a single layer. Thus it may be said that the batts are not only narrow, they are also thin. There is another reason for supporting each wheel 35 by means of a plurality of batts. A batt in the form of a single thick plate or even in the form of a pair of thin plates superimposed upon each other will warp after a number of cycles of heating and cooling. In order to produce grinding wheels with plane sides these grinding wheels should have flat, that is to say plane surfaces to rest upon during vitrification. Another feature of the support for the wheels is the laying of the upper layer of batts 32 across 45 instead of along the lower layer of batts 30. This helps to produce a level flat surface for supporting the wheel 35.

Referring to Figure 2, it will be seen that the batts 30 have a groove 36 at one end and a tongue 37 at the other end. These batts extend the entire length of the kiln in a long line of batts. They are pushed through the kiln by a force applied against the end batt at the entrance end of the kiln. Consequently each batt 30 is firmly pressed against adjacent batts and the tongue and groove junction will hold a broken batt in place if the adjacent batts are still whole. Preferably also the upper batts 32 have tongues and grooves as shown in Figure 3. As will be noted by reference to Figures 2 and 3, the batts

30 are thicker than the batts 32. Since the batts 30 are the ones which span the tunnel they are the primary conveyors of the load.

Figures 4 and 5 illustrate respectively a longitudinal section and a cross section of a tunnel kiln in which the refractory supports of the invention can be used. This tunnel kiln has a rectangular parallelepipedal box structure comprising steel side plates 40, steel bottom plates 41, and steel top plates 42. To the side plates 40 are secured steel legs 43 and to the bottom plates 41 are secured a number of centerline legs 44. The bottom plates 41 are braced with angle irons 45 and the top of the kiln is strengthened by cross beams 46.

Resting on the bottom plate 41 in the firing zone of the kiln is a mass 50 of refractory bricks forming a generally rectangular parallelepipedal structure the top face 51 of which is the bottom of the tunnel 52. This mass 50 stops just short of the side plates 40 leaving spaces which are filled with refractory insulating powder such as porous silica 53.

Bricks 54 continue the structure upwardly on either side of the tunnel 52 and large bricks 55 continue the structure still further upwardly, the bricks 54 and 55 forming vertical side walls 56 of the tunnel 52 and also inclined walls 57 of the tunnel 52.

Secured to the side plates 40 are long angle irons 60 which support channel irons 61 (Figure 4) arranged in pairs. Each pair of channel irons 61 helps to support two courses of roof bricks 62. Stating this in another way, two channel irons 61 whose open sides are opposite each other support between them a course of roof bricks 62 extending clear across the kiln. These roof bricks 62 in the firing zone are short to give room for the combustion tubes and the burners; roof bricks 62a are cut away as shown while roof bricks 62b are long to bring down the roof of the tunnel close to the ware and the baffles 33 and 34. In the preheating zone and in the annealing zone roof bricks 62b are used.

As will clearly be seen, porous silica 53 is located in spaces adjacent the side plates 40 up to the top of the kiln and there is more porous silica 53 on top of the roof bricks 62, 62a and 62b.

Supported by the bricks 55 are bricks 65 having bores to receive refractory tubes 66 on one side of the kiln in which are burners 67. On the other side of the kiln opposite a burner 67 the bores in the bricks 65 receive refractory flue tubes 68 and short refractory tubes 69 in which are plugs 70.

Similarly, in the mass of bricks 50 are bricks 65 having bores receiving refractory tubes 66 in which are burners 67, the bores in the bricks 65 also alternately having refractory flue tubes 68 and short refractory tubes 69 plugged with plugs 70. The tubes 66 and 68 are connected by combustion tubes 75. The arrangement of burners and flue tubes 68 is alternate both horizontally and vertically. That is to say on either side of a burner 67 there is a flue tube 68 and below a burner 67 is a flue tube 68, etc.

Connections 76 connect the burners 67 to piping, not shown, which piping is connected up to sources of gas and air under pressure in order to supply the burners 67 with combustion gases. The gases burn mostly in the combustion tubes 75 which, for example, can be made of bonded silicon carbide and which become very hot. The combustion gases from the refractory flue tubes 68 go into flues 78 in the bricks 50, 54 and 55

whence they lead to flues, not shown, to preheat the preheating zone of the kiln. Since this invention relates to the refractory supports for the ware, I do not deem it necessary to describe the entire kiln, and enough of the structure of the kiln has been described so that the utility of the invention may be readily apparent.

The rods 31 may be located in grooved elongated refractory members 80 which form part of the bottom of the tunnel 52 of the kiln in the firing zone; elsewhere the batts 30 may ride upon rollers, not shown. The batts 30 have wide grooves 81 at either end so that they will not slip off the rods 31 nor off the rollers, not shown. In the operation of this kiln the operator from time to time places an additional load in front of the entrance end and then causes a ram to push the new load against the last previous load to be introduced and this pushes all the loads ahead of it moving every load the distance of one section in the kiln and causing one load to move out of the exit end of the tunnel. The assembly of batts 30 and 32 with the baffles 33 and 34 and a grinding wheel 35 constitutes a unit load. A unit load has a length just equal to one section of the kiln and one section of the kiln is the distance between successive legs 43.

For annealing purposes the batts 30 and 32 may have cut-outs to form a hole 82 in each unit load to allow air to move upwardly through the refractory support in the annealing zone of the kiln.

A solid batt of the overall dimensions of the composite support of the invention would quickly go to pieces in a tunnel kiln of the type described operating at a top temperature of 1200° C. But the composite structure of refractory support for wheels to be vitrified enables a tunnel kiln of the type illustrated to be successfully operated. It will readily be seen that this type of tunnel kiln is efficient because the entire supporting means for the ware to be vitrified has a mass not greatly in excess of the ware to be vitrified in contra distinction to the usual tunnel kiln where the cars and refractory supports have a mass many times that of the ware to be vitrified. Furthermore, the baffles 33 and 34 substantially seal off each section of the kiln from every other section of the kiln and thus optimum preheating, firing and annealing conditions can be achieved. That is to say, at a given time the entire area of the wheel 35 is subject to the same temperature conditions. There is one exception to the foregoing statement, namely that deliberately during the annealing the wheels are cooled from the inside to the outside thus to take advantage of the reverse strain annealing described and claimed in U. S. Letters Patent No. 2,034,721 to my colleague W. L. Howe dated March 24, 1936. However, so far as the broad features of this invention are concerned, the holes 82 can be omitted and very satisfactory vitrified wheels nevertheless can be produced. The baffles 33 and 34 not only protect the wheels 35 from temperature gradients during all the stages of vitrification, viz. preheating, firing and annealing, but they also protect the batts 30 and 32 from such temperature gradients and even protect themselves. By providing these baffles 33 and 34 there is very little difference of temperature from one part to another of any given section of the kiln tunnel 52 although there are predetermined differences of temperature between any two sections.

Batts are customarily made of materials that are matured to a strong condition at tempera-

tures higher than those experienced by the batt in use. This gives a product having maximum stability in use against change in dimensions, etc. It is advantageous to employ materials of as low expansivity as feasible so as to reduce the amount of dimensional change and resulting stress as a function of temperature change. Batts and other kiln furniture have long been made of refractory fire clays. These give products of satisfactory expansivity characteristics but of relatively low strength and low heat conductivity. Silicon carbide as the main ingredient of batt mixtures gives improved products because in addition to low expansivity they have high strength and high heat conductivity. Likewise, batts composed of mullite may have been essentially originally of the electric furnace fused variety, or may have been developed by the maturing operation to which the batt was subjected in manufacture, have advantages over fire clay batts. Furthermore, refractory batts for very high temperature use may now be made as sintered or recrystallized products, often substantially bondless, many of which may be classed as pure oxide refractories. The refractory supports for ware according to this invention are preferably made of bonded silicon carbide but so far as the broader features of my invention are concerned they may be made of other refractory materials.

As an example of a bonded silicon carbide composition for batts according to the present invention, I may make a mixture according to the following formula:

*Example*

| Material:                                   | Parts by weight |
|---------------------------------------------|-----------------|
| No. 14 to No. 24 grit size silicon carbide  | 45              |
| No. 30 to No. 90 grit size silicon carbide  | 25              |
| No. 100 grit size and finer silicon carbide | 18              |
| Ball clay                                   | 12              |
| Dextrine powder                             | 2               |
| Rye flour                                   | 1               |
| Water                                       | 4               |
| Total                                       | 107             |

The silicon carbide is the ordinary black grade and is put into a mixing machine of conventional type and the dextrine is added. After mixing for a minute or two the water is added and mixing is continued for a minute or two more. Then the ball clay and rye flour are screened into the mix together and the mixing is continued for five minutes more. This procedure produces a damp granular mixture that is suitable for tamping or pressing. This mixture is then molded in molds shaped to produce the batts and baffles of the shapes shown, and then the "green" batts and baffles are fired in a suitable kiln at a temperature substantially higher than the highest temperature which will be found in the kiln in which they will be used. For example, if the firing zone of the tunnel kiln herein described is heated to a temperature of 1250° C., the batts and baffles should be fired to a top temperature of at least about 1400° C.

It will thus be seen that there has been provided by this invention refractory supports for ware in a tunnel kiln in which the various objects hereinabove set forth together with many thoroughly practical advantages are successfully achieved. As many possible embodiments may be made of the above invention and as many changes might be made in the embodiment above set forth, it is to be understood that all matter hereinbefore set forth or shown in the accom-

panying drawings is to be interpreted as illustrative and not in a limiting sense.

I claim:

1. A batt assembly comprising a pair of parallel rods, a plurality of rectangular batts with grooves on the undersides and having dovetailed edges in contiguous relation with the dovetails in engagement and with the grooves on the rods, and a second plurality of rectangular batts positioned in contiguous relation transverse to and resting upon the first plurality of rectangular batts.
2. In a batt assembly as claimed in claim 1, the combination with the parts and features therein specified of a pair of baffles on said second plurality of batts.
3. An assembly of batts comprising a plurality of rectangular batts with dovetailed edges said batts being located in a plane with the dovetails in engagement, a second plurality of rectangular batts resting cross-ways upon said first plurality of rectangular batts, and a pair of baffles with concavely curved edges resting upon said second plurality of batts, the planes of the curves of the concavely curved edges of the baffles being parallel to the planes of both pluralities of batts and the baffles being located on the second plurality of batts so that the curved edges face each other.
4. In a batt assembly as claimed in claim 3, the combination with the parts and features therein specified of the further feature that each of said baffles consists of a plurality of separate parts.
5. A refractory support for ware in a tunnel kiln comprising two lines of rods said lines being parallel, a plurality of unit loads resting on said rods, each load consisting of a plurality of rectangular batts having grooves on the underside resting upon said rods with the rods being located in the grooves, dovetailed means in each edge of each batt which runs perpendicular to the lines of rods, all of the batts being in dovetailed engagement in a load and from load to load, and in each load an additional plurality of rectangular batts resting upon the first described batts said additional batts extending generally in the same direction as the rods.
6. In a refractory support for ware in a tunnel kiln as claimed in claim 5, the combination with the parts and features therein specified of a pair of baffles having concavely curved edges in each unit load the concavely curved edges of the baffles facing each other thus to provide an insulated space for a grinding wheel to be vitrified.
7. In a refractory support for ware in a tunnel kiln as claimed in claim 6, the combination with the parts and features therein specified of the additional feature that each baffle is in three parts.

GEORGE N. JEPPSON.

REFERENCES CITED

The following references are of record in the file of this patent:

65 UNITED STATES PATENTS

| Number       | Name     | Date           |
|--------------|----------|----------------|
| 971,160      | Vance    | Sept. 27, 1910 |
| 979,425      | Butler   | Dec. 27, 1910  |
| 70 1,262,010 | Brownlee | Apr. 9, 1918   |

FOREIGN PATENTS

| Number | Country       | Date |
|--------|---------------|------|
| 6,139  | Great Britain | 1914 |